

## UNITED STATES PATENT OFFICE

2,305,034

## COMPOUNDED PETROLEUM OIL

Raphael Rosen, Elizabeth, and Ben W. Geddes,  
Linden, N. J., assignors to Standard Oil De-  
velopment Company, a corporation of Delaware

No Drawing. Application December 20, 1939,  
Serial No. 310,172

18 Claims. (CL 252—47)

The present invention relates to addition agents which inhibit the oxidation of petroleum oils and more specifically to compounded lubricating oils containing such addition agents.

It has been proposed to use as addition agents for increasing oxidation resisting qualities of mineral oils certain basic organic nitrogen compounds, characterized by having a heterocyclic structure containing nitrogen. Compounds of this type occur in petroleum products which have been heated to distillation temperatures. While these compounds when used alone do inhibit oxidation to a certain extent, it has been found that considerably greater oxidation resisting power is conferred upon an oil when the element sulfur is in some manner added to the oil with the nitrogen base.

The addition of sulfur may be accomplished in various ways. One way is to sulfurize the nitrogen base directly, as, for example, by heating the base with sulfur, or by treating the base with sulfur dichloride in a suitable solution. The sulfurized nitrogen base is then added to the mineral oil.

Another and somewhat more effective method of adding sulfur to the nitrogen base antioxidant is to add to the oil, along with the base, a sulfur-containing organic compound, preferably one which is itself a mineral oil oxidation inhibitor. The manner in which the base and the sulfur or sulfur-containing organic compound cooperate to give superior antioxidant effects is not understood; but it has been found as a matter of experience that an oil treated in the manner described has considerably greater oxidation resisting power than is indicated by the summation of the known effects of the two ingredients when used separately. For example, a given weight of a mixture of approximately equal parts of a nitrogen base extracted from petroleum and a sulfurized polymer of isobutylene will give a much greater antioxidant effect in an oil than an equal weight of either one of the materials alone.

Petroleum oils of all boiling point ranges are susceptible to improvement in oxygen resisting characteristics by the use of the addition agents herein described. These include kerosenes, Diesel oils, transformer oils, lubricating oils and the like; but the invention is of particular value in the production of lubricating oils which resist oxidation at normal internal combustion engine temperatures, and in the preparation of lubricating greases containing mineral oils.

The nitrogen base compound which is employed as the basic addition agent may be any

5 organic compound of base characteristics having a heterocyclic ring structure containing nitrogen. Compounds of this type include, as examples, quinoline or acridine, or the alkyl or aryl derivatives of these compounds, or of pyridine. More especially preferred are the naphthenic bases, i. e., those containing a hydroaromatic ring with an atom of nitrogen in such ring. Such compounds include substances of the type of alkylated piperidine, or the more complex basic materials obtained from petroleum distillates. 10 It is desirable to employ compounds having boiling points above 300° F. at atmospheric pressure, and in the case of lubricating oil blends the addition agent should ordinarily have a boiling point above 350° F.

Convenient and economical sources of the preferred nitrogen bases of the present invention are the distillates obtained in the rectification of petroleum or shale oil. The asphaltic petroleums of California are particularly rich in nitrogen compounds, having a nitrogen content in the neighborhood of 1%. It has been found, however, that nitrogen bases are not contained in 15 the crude oils, but are formed on heating the crude oils to the temperatures encountered in distillation processes, i. e., temperatures varying from 275° F. to 740° F. Cracking temperatures are less favorable, but do generate basic nitrogen 20 compounds to some extent. Naphthenic bases obtained from California petroleum are predominantly of hydroaromatic character, but contain also a smaller percentage of aromatic bases. The compounds present have a varying and complex 25 structure, but they consist only of carbon, hydrogen and nitrogen, the nitrogen being present in a heterocyclic ring.

The nitrogen bases may be separated from the 30 oils by extraction with agents such as liquid sulfur dioxide, hydrochloric acid or sulfuric acid. By one convenient method of preparing the bases, a kerosene fraction obtained by the fractional distillation of a California asphaltic crude oil is extracted at about —7° C. with liquid sulfur 35 dioxide. The mixture so obtained is heated to about 38° C. under 75 pounds pressure to evaporate off the excess sulfur dioxide, cooled and extracted with cold water to obtain an aqueous solution of acid sulfites of nitrogen bases. The 40 aqueous solution is further heated to remove as much sulfur dioxide as possible, the remaining sulfur dioxide being removed in a rectifying column, and an aqueous solution of sodium hydroxide is added to the purified aqueous solution 45 to liberate the bases. The latter separate as

oily layer and are removed in a separator and fractionally distilled to obtain a crude mixture of nitrogen bases, which may, if desired, be redistilled under high vacuum to secure pure narrow cuts.

The sulfur-bearing antioxidants which are added to the petroleum oils, in addition to the nitrogen bases, according to the preferred mode of carrying out the present invention, are any sulfur-bearing organic materials which impart oxidation resisting properties to such oils. Such materials include compounds of simple and well known composition, such as the alkyl phenol sulfides or polysulfides or their metallic salts, e. g. tertiary amyl diphenol sulfide and the aluminum salt of di-tert-butyl diphenol sulfide, also 10 dialkyl and diaryl polysulfides, e. g., diethyl tetrasulfide and dibenzyl disulfide, and mercaptans, e. g., benzyl mercaptan, as well as organic thiophosphites, e. g., amyl phenyl thiophosphite.

Other suitable antioxidants are those sulfurized oils obtained by heating fatty or mineral oils in the presence of sulfur or sulfurizing agents, such as sulfur chloride, according to well known means.

Certain hydrocarbons, specifically polymers of low molecular weight olefins, particularly those having less than six carbon atoms, such as ethylene, propylene, butylenes and amylenes, are superior materials for sulfurization, in that the sulfurization may be accomplished with very little cracking or polymerization, and without the production of darkly colored or otherwise objectionable constituents. Of these materials particularly satisfactory are the polymers of isobutylene and isoamylene in that these materials instead of cracking merely depolymerize to a certain extent during the sulfurization treatment and therefore give rise to cleaner and more desirable products. Materials of this kind are therefore especially suited for blending in lubricating oils and aiding in the inhibition of autoxidation.

The polymers which are disclosed above, and particularly the polymers of isolefins, boil above 100° C., and preferably from about 150° to about 275° C. These materials may be made by polymerization of various olefins or mixed olefins, using catalysts such as sulfuric or phosphoric acid, aluminum chloride, zinc chloride, boron fluoride, or other similar active halide catalysts of the Friedel-Crafts type. In addition to these, various siliceous catalysts may also be used, such as fuller's earth or clays, especially clays activated by treatment with mineral acids, such as sulfuric, phosphoric, hydrochloric or hydrofluoric acids. Copolymers, also suitable for use in this invention, are formed by the polymerization of mixtures of olefins, preferably an isolefin, such as isobutylene, with the other olefins, such as normal propenes, butenes or pentenes of the same or a different number of carbon atoms per molecule. The particular methods of producing the polymers and copolymers are well known and form no part of the present invention.

The present invention includes the use, as one of the addition agents which aid in the lowering of the oxidizing tendencies of petroleum oils, of the sulfurized products of the above described polymers. A suitable method for conducting the sulfurization is by heating the polymer or mixture of polymers with free sulfur at an elevated temperature and maintaining the temperature for a prolonged period. Sulfurization begins at

about 180° C. and is quite vigorous within the range from 200 to 250° C. The time of heating is governed by the temperature, lower temperatures requiring a longer time, but ordinarily it should not be in excess of 15 minutes at the upper end of the temperature range given above, and the preferred temperature range depends upon the boiling point of the reactants, and usually a temperature of 180° to 250° C. is desirable. The sulfur combines with the hydrocarbon polymer quite readily with an evolution of hydrogen sulfide.

5 The product produced above may be blown to eliminate hydrogen sulfide and washed and low boiling constituents may be evaporated or distilled off with steam. In many cases a small amount of sulfur is present which has not reacted, and this may be separated by filtration or otherwise, and after this is done the filtrate is stable and sulfur does not precipitate or settle out.

15 The polymers described above may also be sulfurized by other suitable methods; for example, they may be heated with sulfur halides, such as sulfur monochloride or sulfur dichloride. The resulting sulfurized polymer will contain small amounts of chlorine, and may be used in this form in lubricating compositions in which the halide is not objectionable. The sulfurized polymer may also be refined with alcoholic alkali to remove the halide.

20 Another method of preparing the sulfurized polymer oil is to heat the polymer with sulfur to 250° C. for between 15 and 20 minutes in the presence of metallic oxides, especially zinc oxide, or with such metallic oxides in admixture with alkyl phenol sulfides, such as tertiary amyl phenol sulfide or disulfide, or compounds which are known to exert an accelerating influence 25 upon the vulcanization of rubber hydrocarbons. Products so obtained are refined by treatment previously mentioned in connection with the preparation of the materials according to other procedures. The advantages of this method of preparation are that less sulfur is lost as hydrogen sulfide, and the time and temperature of the reaction are appreciably reduced.

25 A particularly valuable application of the present invention is the use of the sulfurized olefins with the nitrogen bases in lubricating oil compositions. A feature of the blending characteristics of the sulfurized polymer oil is that it causes little impairment of color or cast. As a matter of fact, the addition of the sulfurized olefin polymer produces a very desirable red color and may be used as a lubricating oil dye. This color effect may be obtained in the presence of nitrogen bases which are also added to the lubricating oils in accordance with the present invention, since a properly refined nitrogen base material will impart little or no color to the oil when used in small quantities as antioxidant. This is an advantage over sulfurized mineral oils which have been previously employed as lubricating oil addition agents in that such materials cause some depreciation in color when blended with lubricating oil stocks.

30 In accordance with the preferred method of carrying out the present invention, a compounded oil is obtained by adding small quantities of both a sulfur-bearing antioxidant and nitrogen bases to the hydrocarbon oil. The effectiveness of the antioxidants is not impaired by the presence in the oil of naturally occurring sulfur or nitrogen.

As to quantities, it has been found preferable to employ such an amount of sulfur-bearing antioxidant as will provide from about 0.0075 to about 0.10%, and more preferably, especially in the cases where a sulfurized polymer oil is used, from 0.0075% to 0.015%, of sulfur in the form of a combination in the antioxidant compound in the finished oil. The sulfur so combined is not to be confused with the sulfur naturally present in the lubricating oil. In other words, when an antioxidant containing about 10% of sulfur is used, such an antioxidant should be added to an oil in quantities varying from about 0.075% to about 1.0%. The nitrogen bases are preferably added in quantities varying from about 0.10% to about 1% or even up to 5% of the oil, a more preferred range being from 0.10% to 0.25%. Where sulfurized nitrogen bases are added as the sole antioxidant, these are likewise preferably added in quantities from about 0.10% to about 1%, or even up to 5%.

It has been found that the addition agents of this invention do not have any detrimental effects on the physical character of the lubricating oil or other mineral oil to which they are added, such as viscosity, gravity and flash point, or on the amount of carbon residue formed on prolonged use of the oil. The present materials may be used as the sole blending agents or they may be added, as in the case of a lubricant, with other ingredients which serve other purposes. They are, for example, useful agents when added to leaded lubricating oils, that is to say lubricants containing lead oleate, lead naphthenate, lead sulfonate or other heavy metal soaps. They also may be added along with oiliness agents, pour depressants, lubricating oil dyes or agents to give fluorescence. They may be used in conjunction with any other antioxidants or with thickeners, sludge dispersers and the like. In the case of Diesel fuels, there may be present ignition promoters and other ingredients common to motor fuels.

As has been stated above, an effective antioxidant for oils, superior to nitrogen bases alone, may be prepared by sulfurizing the nitrogen bases directly. The sulfurized products may be obtained, for example, by heating the bases with sulfur, or by treating the bases with sulfur dichloride in a suitable solution. The sulfurized products may be purified by treatment with sodium sulfide solution to improve the color and to render them comparatively non-corrosive. Such purification lowers the sulfur content somewhat. The final product lowers the oxygen absorption rate of a lubricating oil with which it is blended to a greater extent than the unsulfurized nitrogen base, but not as much as does a combination of a sulfur-bearing antioxidant, such as a sulfurized polymer oil, and a nitrogen base, which is the preferred embodiment of the present invention.

The value of the antioxidants of the present invention when used in lubricating oil blends have been determined by a standard oxygen absorption test. This test is used for the most part in judging the oxidation susceptibility of a lubricating oil at engine operation temperatures. A known amount of oxygen is bubbled through 10 cc. of the lubricating oil maintained at 200° C. The oxygen is continuously recycled. At the end of successive 15 minute periods the amount of oxygen absorbed by the oil is measured. The results, usually termed the oxidation rate of the oil, are given as the number of cubic centimeters

of oxygen absorbed by 10 cc. of an oil per 15 minute intervals at 200° C.

In the following examples, methods of preparing a sulfurized polymer oil, nitrogen bases and blends of these with lubricating oils are shown, together with data on the oxidation rates of oils containing such materials:

*Example 1*

10 An isobutylene polymer having a viscosity of 84 seconds Saybolt at 210° F. and open cup flash point of 305° F. was caused to react with 15% of sulfur by heating to 250° C. for about 15 minutes in the presence of 1% of zinc oxide and 1% of "Pip-Pip" (piperidinium-pentamethylene-di-thiocarbamate), a commercial vulcanization accelerator manufactured by the Monsanto Chemical Company. The product obtained by this method had a sulfur content of 6.45%.

*Example 2*

An oxygen absorption test, conducted according to the standard procedure described above, was made on a blend consisting of a refined mineral lubricating oil of 20 S. A. S. grade to which had been added 0.125% by weight of a sulfurized polymer oil prepared according to Example 1 and 0.125% of a nitrogen base product prepared by the extraction of a kerosene fraction of a California crude petroleum, the base used being a fraction boiling at 145-165° C. at 4 mm. pressure and containing about 4.5% nitrogen. Corresponding oxygen absorption tests were made on a sample of the unblended base oil, also on samples of this oil containing the same nitrogen base material alone, also the sulfurized polymer oil alone, and a sample blended with a sulfurized nitrogen base containing 1.66% of sulfur. The data of the following table show the number of cubic centimeters of oxygen absorbed by 10 cc. samples of the oils for several successive 15 minute intervals at 200° C.

|                                                                      | Oxygen absorption rate |         |
|----------------------------------------------------------------------|------------------------|---------|
|                                                                      | 15 minute intervals    | Average |
| 45                                                                   |                        |         |
| Base oil                                                             | 81, 36, 26             | 48      |
| Base oil+0.25% of nitrogen bases                                     | 57, 30, 23, 21         | 33.8    |
| 50 Base oil+0.25% of sulfurized polymer oil                          | 56, 46, 30, 26         | 39.5    |
| Base oil+0.25% of sulfurized nitrogen bases                          | 39, 20, 16, 16         | 20.5    |
| 55 Base oil+0.125% each of sulfurized polymer oil and nitrogen bases | 3, 9, 13, 11           | 9       |

The present invention is not to be considered as limited in any way by any of the herein described examples, which are given by way of illustration only, but is to be limited solely by the terms of the following claims in which it is desired to claim all novelty inherent in the invention.

We claim:

1. An improved mineral oil composition comprising a petroleum oil fraction, a small proportion, not more than 5%, of an organic base having a heterocyclic structure containing nitrogen, said organic base being an antioxidant for petroleum oils, and a small proportion, not greater than 0.1%, of the element sulfur, said sulfur being present in an organic compound which is an antioxidant for petroleum oils.

2. An improved mineral oil composition comprising a petroleum oil fraction, a small proportion, not more than 5%, of an organic heterocyclic nitrogen base extracted from a petroleum

distillate, said nitrogen base being an antioxidant, and a small proportion of a sulfur-bearing organic antioxidant, the amount being sufficient to produce a concentration of not more than 0.1% of sulfur in the form of the said sulfur-bearing antioxidant.

3. An improved mineral oil composition comprising a petroleum oil fraction, a small proportion, not more than 5%, of an organic base having a heterocyclic ring structure containing nitrogen, said organic base being an antioxidant, and a small proportion of a sulfurized polymer of an olefin, sufficient to produce a concentration of not more than 0.1% of sulfur in the form of the sulfurized polymer.

4. An improved mineral oil composition comprising a petroleum oil fraction, a small proportion, not more than 5%, of an organic base having a heterocyclic hydroaromatic ring structure containing nitrogen, said organic base being an antioxidant, and a small proportion of a sulfurized polymer of an olefin, sufficient to produce a concentration of not more than 0.1% of sulfur in the form of the sulfurized polymer.

5. An improved mineral oil composition comprising a petroleum oil fraction, a small proportion, not more than 5%, of an organic heterocyclic nitrogen base extracted from a petroleum distillate, said nitrogen base being an antioxidant, and a small proportion of a sulfurized polymer of an olefin, sufficient to produce a concentration of not more than 0.1% of sulfur in the form of the sulfurized polymer.

6. An improved lubricant comprising a hydrocarbon lubricating oil, a small proportion, not more than 5%, of an organic nitrogen base having a heterocyclic structure and having been extracted from a petroleum distillate, said nitrogen base being an antioxidant, and a small proportion of a sulfurized polymer of an olefin, sufficient to produce a concentration of not more than 0.1% of sulfur in the form of the sulfurized polymer.

7. An improved lubricant comprising a hydrocarbon lubricating oil, a small proportion, not more than 5%, of an organic nitrogen base having a heterocyclic structure and having been extracted from a petroleum distillate, said nitrogen base being an antioxidant, and a small proportion of a sulfurized polymer of an olefin having less than six carbon atoms, sufficient to produce a concentration of not more than 0.1% of sulfur in the form of the sulfurized polymer.

8. An improved lubricant comprising a hydrocarbon lubricating oil, a small proportion, not more than 5%, of an organic heterocyclic nitrogen base extracted from a kerosene fraction of a California asphaltic base crude petroleum oil, said nitrogen base being an antioxidant, and a small proportion of a sulfurized polymer of an olefin having less than six carbon atoms derived by sulfurizing an olefin polymer having a boiling point above 100° C., the amount being sufficient to produce a concentration of not more than 0.1% of sulfur in the form of the sulfurized polymer.

9. An improved lubricant comprising a hydrocarbon lubricating oil, a small proportion, not more than 5%, of an organic heterocyclic nitrogen base extracted from a kerosene fraction of a California asphaltic base crude petroleum oil, said nitrogen base being an antioxidant, and a small proportion of a sulfurized polymer of isobutylene, sufficient to produce a concentration of not more

than 0.1% of sulfur in the form of the sulfurized polymer.

10. An improved lubricant comprising a hydrocarbon lubricating oil, a small proportion, not more than 5%, of an organic heterocyclic nitrogen base obtained by extracting a kerosene fraction of a California asphaltic base crude petroleum oil with liquid sulfur dioxide, said nitrogen base being an antioxidant, and a small proportion of a sulfurized polymer of isobutylene, sufficient to produce a concentration of not more than 0.1% of sulfur in the form of the sulfurized polymer.

11. An improved lubricant comprising a hydrocarbon lubricating oil, a small proportion, not more than 5%, of a fraction of an organic heterocyclic nitrogen base material obtained by extracting a kerosene fraction of a California asphaltic base crude petroleum oil with liquid sulfur dioxide, said fraction of nitrogen base material having antioxidant properties and having a distillation range of about 145° to about 165° C. at 4 millimeters pressure, and a small proportion of a sulfurized polymer of isobutylene derived by sulfurizing an isobutylene polymer having a boiling point from 150° to 275° C., sufficient to produce a concentration of not more than 0.1% of sulfur in the form of the sulfurized polymer.

12. An improved mineral oil composition comprising a petroleum oil fraction, 0.10% to 1% by weight of an organic heterocyclic nitrogen base extracted from a petroleum distillate, said nitrogen base being an antioxidant, and an amount of a sulfur-bearing organic antioxidant sufficient to give the component oil 0.0075% to 0.10% by weight of sulfur combined in said antioxidant.

13. An improved lubricant comprising a hydrocarbon lubricating oil, 0.10% to 1% by weight of an organic heterocyclic nitrogen base material obtained by extracting a kerosene fraction of a California asphaltic base crude petroleum oil with liquid sulfur dioxide, said nitrogen base material having antioxidant properties, and an amount of a sulfurized polymer of isobutylene sufficient to give the compounded oil 0.0075% to 0.10% by weight of sulfur combined with olefin polymer, said sulfurized polymer being formed by sulfurizing an isobutylene polymer having a boiling point from 150° to 275° C.

14. An improved lubricant comprising a hydrocarbon lubricating oil, 0.10% to 0.25% by weight of a fraction of an organic heterocyclic nitrogen base material obtained by extracting a kerosene fraction of a California asphaltic base crude petroleum oil with liquid sulfur dioxide, said fraction of nitrogen base material having antioxidant properties and having a distillation range from about 145° to about 165° C. at 4 millimeters pressure, and an amount of a sulfurized polymer of isobutylene sufficient to give the compounded oil 0.0075% to 0.015% by weight of sulfur combined with olefin polymer, said sulfurized polymer being formed by sulfurizing an isobutylene polymer having a boiling point from 150° to 275° C.

15. An improved mineral oil composition comprising a petroleum oil fraction, and a small proportion, not more than 5%, of a sulfurized organic base, said base having a heterocyclic structure containing nitrogen and having antioxidant properties, the amount being sufficient to produce a concentration of not more than 0.1% of sulfur in the form of the sulfurized organic base.

16. An improved mineral oil composition comprising a petroleum oil fraction and a small proportion, not more than 5%, of a material obtained

by sulfurizing an antioxidant consisting of an organic heterocyclic nitrogen base extracted from a petroleum distillate, the amount being sufficient to produce a concentration of not more than 0.1% of sulfur in the form of the sulfurized nitrogen base.

17. An improved lubricating oil composition comprising a petroleum lubricating oil fraction, a small proportion, not more than 5%, of an organic base containing carbon, hydrogen and nitrogen, but substantially free from halogen, and having a heterocyclic structure containing nitrogen, said organic base being an antioxidant for petroleum oils, and a small proportion, not greater than 0.1%, of the element sulfur, said sulfur

being present in an organic compound which is an antioxidant for petroleum oils.

18. An improved lubricant comprising a hydrocarbon lubricating oil and a small proportion, not more than 5%, of a material obtained by sulfurizing an antioxidant consisting of an organic heterocyclic nitrogen base extracted from a kerosene fraction of a California asphaltic base crude petroleum oil with liquid sulfur dioxide, the amount of the sulfurized nitrogen base present being sufficient to produce a concentration of not more than 0.1% of sulfur in the form of such sulfurized nitrogen base.

RAPHAEL ROSEN.  
BEN W. GEDDES.